

March 23, 1948.

F. F. POLLAK

2,438,349

BENDING OF CORKWOOD

Filed April 28, 1944

2 Sheets-Sheet 1

Fig. 1.



Fig. 2.



INVENTOR.

Frederick F. Pollak  
BY *Lebecum*  
ATTORNEY

March 23, 1948.

F. F. POLLAK

BENDING OF CORKWOOD

2,438,349

Filed April 28, 1944

2 Sheets-Sheet 2

Fig. 3.



Fig. 4.



INVENTOR.

BY *Frederick F. Pollak*

*J. E. Freeman*

ATTORNEY

## UNITED STATES PATENT OFFICE

2,438,349

## BENDING OF CORKWOOD

Frederick F. Pollak, New York, N. Y.

Application April 28, 1944, Serial No. 533,219

5 Claims. (Cl. 144—309)

1

This invention relates to important developments of the methods for the treatment of corkwood, balsawood and similar light woods disclosed in my copending patent application Ser. No. 527,505.

This application is based on the recognition that corkwood and particularly its lightest representative, the balsawood, undergoes a remarkable and astonishing alteration of its properties if subjected to certain comparatively simple treatments and particularly to compression, swelling and drying; the structure and the texture of the wood is thereby entirely changed; the previously fragile and easily breakable wood is in this manner converted into a material which is well usable for many purposes and particularly also as a constructional and building material.

The present invention is an important supplement in this respect, and it is the main object to bend corkwood and balsawood into desired arcuated shapes.

It is also an object of the invention to produce uniformly and symmetrically bent balsawood workpieces and to avoid irregularities of the final form.

It is a particular object of the invention to produce from corkwood and balsawood perfect circular and part-circular articles.

It is also an object of the invention to combine with the bending of the wood treatments which improve its properties and particularly increase its strength and hardness.

It is a further object of the invention to establish the principles which permit the creation of faultless bends and, therefore, assure the production of highly usable bent corkwood and balsawood articles.

Further objects and purposes of my invention will be apparent from the following description in conjunction with the attached drawing of

40

Fig. 1 is a vertical sectional view of a bending mold to be used in the performance of this invention.

Fig. 2 is a top view of the mold.

Figs. 3 and 4 are sectional views of the working members of the mold and of the workpiece in an intermediary and in the final stage of the bending operation.

As generally known, the shaping of wood by bending is a rather difficult problem. In order to bend wood into curved and arcuated bodies, for instance, into circular or part-circular articles, the dried but otherwise mechanically untreated wood is subjected to the individual or the com-

50

bined action of heat, steam and pressure; a certain bending action may also be imparted to wood by mere pressure and without the application of heat or steam.

5 This situation, however, is entirely diverse in the case of corkwood and balsawood; these types of light wood cannot be bent to any appreciable degree in their original state; only by a compound with veneers and due to the support created thereby a limited bending of corkwood and balsawood may be accomplished.

The non-bendability is caused by the peculiar structure and texture of these light wood types.

15 As explained in my former application the corkwood and particularly the balsawood may well be identified as an extremely unyieldable and stiff agglomeration of hollow longitudinally orientated comparatively short fibers, similar in their characteristics to short straw halms which are united by transverse bands, the interstices between the hollow fibers being partly filled with incrustation masses.

20 If balsawood is compressed by pressure acting vertically to the longitudinal direction of the hollow fibers, the transverse structure supporting elements are disrupted and probably freed on the one side from their compound with the longitudinal fibers, whereas the union on the other side remains unaltered; when the compressed balsawood is swelled up by imbibition, the transverse supports seem to assume their former location and to impart to the main fibers a support which is similar to the one which existed in the initial state; the swelled up bodies do not materially change their shape by drying.

25 This basic observation is utilized according to the instant invention for bending balsawood and the previously made statement that balsawood cannot be bent to any appreciable degree is now supplemented insofar as a bending against the direction of the fibers is entirely impossible; even the slightest attempt in this respect is bound to be a failure, since the fibers are utterly fragile and are immediately ruptured and broken if the

30 least bending stress is imparted thereto; slight arcuated deformations are only obtainable in the direction of the fibers and seem to be the result of a bending of the transverse bands and not of the fibers.

35 Furthermore, it must be kept in mind that the bending of a body involves an elongation of its outside layers and a compression of the layers which are located at its inside. The displacement of the particles in these various layers takes place under an angle in relation to the center

line of the curvature and the magnitude of this angle is a factor which greatly influences the bending procedure.

It might be well assumed that a further increase of the natural softness of the wood would satisfy these conditions and favorably influence the bendability of the wood under the provision that its inner coherence would be preserved.

I found that this object may be accomplished by compressing the wood to about one-fifth to one-tenth of its initial thickness and reswelling the same through imbibition with boiling water to about 50 to 90% of its original thickness. The softness and pliability of the balsawood is thereby increased and a bending at least to a 15 limited extent was rendered possible.

Further experimentation, however, proved that the thus produced bendings were irregular and that, for instance, satisfactory circular or part-circular workpieces could not be obtained.

I realized that sufficient softness and pliability might not be the only influencing factor in the art of bending balsawood and that the displacement of each individual particle of the softened balsawood and the length of the way might have 20 to be considered which each particle must travel during the bending operation.

Furthermore, I conceived that the extent of this displacement would be directly related to the thickness of the balsawood workpieces. If, for instance, two boards of a different thickness are bent into circular and part-circular bodies, the incurvation at the circumference of the thicker body will be larger and every particle of this body must travel a longer way during the bending operation; it thus became apparent that in addition to the softness of the balsawood the thickness of the workpieces influences the bendability; as a natural consequence of this mental analysis the advisability arose to subject the balsawood to high compression and to reduction of its original volume to thin pieces before subjecting the same to further treatment.

In the practical realisation of this principle it was found that balsawood sheets upon compression by a high pressure of about 2000 lbs./sq. inch to  $\frac{1}{8}$  inch from about 10 times their original thickness could be comparatively easily bent by means of a suitable mold. If the bent objects are then immersed in water, swelled-up and dried in the mold at a temperature of about 110° C., the bent pieces retain their shape even when re-immersed in water.

In order to produce thicker articles several bent bodies were superposed, glued and pressed together. This method, however, resulted in a 55 breakage of the bent pieces.

Only at this state of my investigations I realized that another peculiar property of the balsawood might have to be considered with regard to bendability, and this is the remarkable inertness of the particles of the compressed wood and their indisposition to move. If balsawood is compressed, the fibers remain in the location 60 imparted thereto by the compression, whereas after all being a wood product, it could be expected that the fibers would resume their former position and shape as soon as the pressure was released.

This observation led to the necessity to perform the bending of the compressed balsawood in such a manner that sufficient time was given to the particles to overcome their natural inertness and to move under the influence of the 65

bending force into new positions; in other words, the necessity arose to bend slowly.

The above recited various observations resulted in the establishment of certain principles with regard to the successful bending of corkwood and balsawood, which are summarized as follows:

1. Cork and balsawood must be strongly compressed and reduced in thickness before the bending is commenced;

2. If sufficiently compressed, the wood can be bent by means of a suitable mold irrespective of its initial thickness, if certain additional precautions are observed;

3. The bending must be performed at a timely rate which permits its particles to establish themselves in the new location resulting from the bending; in other words, the bending must be performed at a slow rate;

4. The bent material must be reswelled and dried in the bending mould.

During my endeavors to produce bodies of greater thickness by uniting strongly compressed bent parts, an observation was made of particularly interesting nature.

25 Three semi-circularly bent thin pieces were superposed upon each other and located in water for reswelling purposes. A small weight was placed on top of the combined body. A lifting of the weight was expected to take place equally to the increase of thickness caused by the reswelling of the three pieces.

However, the weight rose far above the precalculated height.

Upon examination of this rather surprising 35 result it was found that the uppermost of the three semi-circular objects had greatly changed its circular form in its center portion and the latter had assumed a somewhat pointed rectangular shape, whereas the two side portions of 40 the same had preserved the circular form. It was obvious that the distortion of the center portion had caused the increase in height over the expected ratio.

45 The lowermost of the three pieces, however, had retained its regular semicircular shape; the center portion of the middle piece showed a change of form lying between the strong deformation of the uppermost piece and the shape preservation of the lowermost piece.

50 The peculiar action and the strong distortion of the uppermost piece was obviously caused by the great swelling pressure exerted upon the same from the outside.

Similar distortions of semi-circular bent pieces 55 were ascertained, when thicker pieces were located for swelling in bending molds, the working surfaces of which had a small radius and an accordingly great incurvation.

When semi-circular bending molds of this type 60 were used for the swelling of the bent pieces, fold-like irregularities and breakages occurred in the center portion of the treated workpieces.

From these observations it appeared that a 65 definite relation exists between the thickness of the compressed balsawood and the extent of incurvation up to which it may be safely bent, and that this bending limit is controlled by the smallest admissible radius of the curve or circle imparted to the compressed balsawood; in other words, the art of bending balsawood articles by compression and reswelling was seemingly governed by a certain direct relation between a maximum thickness of the compressed workpieces 70 and a minimum bending radius which is the ra-

dius of the inner final incurvature imparted to the workpiece by bending; this ratio must be maintained unless irregularly bent pieces or breakages will result.

Needless to point out that balsawood workpieces which in the light of the above explained theory had been improperly treated would have a weak spot in their center portion and, therefore be not usable for most purposes and particularly not for constructional work and for building and similar purposes.

Based on the above explained principles and purposes of this invention the bending of balsawood will now be described in detail with reference to the accompanying drawing.

A rectangular board 4 was cut from air-dried balsawood; due to its softness the wood can be easily cut into desired shapes by means of ordinary cutting or similar tools.

The board is charged between the plane platens of a customary, for instance hydraulic press and compressed at room or a slightly elevated temperature for a period of several minutes at a pressure which may be advantageously maintained between 1000 and 3000 lbs./sq. inch or more.

The board is thereby compressed up to about  $\frac{1}{10}$  of its original thickness without otherwise undergoing a change of its shape; the compressing conditions will vary with the size of the workpieces and the degree of compression.

The equipment used for bending the compressed balsawood board 4 is composed of a lower tubular circular mold member 1 made of a sufficiently hard material, such as steel.

This mold member 1 is provided with two series of bores 3 adjacent to its lower two edges. Threaded bolts 3 are located in these bores; the bolts carry at their upper ends a thin plate 2 of a flexible strong material, for instance flexible steel.

The bending mold is situated in a vessel 5 provided with a feed pipe 6 and a discharge pipe 7.

The compressed balsawood board 4 is placed between the two members 1, 2 of the bending mold, as shown in Fig. 1.

The bolts are gradually tightened by screws 9 and plate 2 is thereby slowly forced into an incurvature; as soon as the plate 2 reaches the board, the latter is bent. The tightening is continued until a distance is reached between the upper and the lower mold members which corresponds to about between 6 to 9 tenths of the thickness of the original board. At this phase of the bending operation the board has been forced into a shape approximately resembling the one shown in Fig. 3, which figure illustrates the second stage of the work.

The previously stated rule must be observed to perform the bending carefully and slowly, as the balsawood particles require a certain time to travel into their new locations in conformity with the gradually changed shape of the board.

Water is now admitted to vessel 5 through tube 6 and the board swells by imbibition; under the influence of the pressure resulting from the swelling the bending of the board continues until it tightly contacts on its outside the mold members 1, 2, assuming at the same time the shape shown in Fig. 4, which shape is identical to the space between the two mold members.

The end shaping by swelling requires approximately 15 minutes, if the initial thickness of the board is about one inch.

It is to be noted that this end shaping is mainly

accomplished by the pressure resulting from the swelling of the wood which is a most desirable working condition.

The mold may be provided with suitable heating means which will render it possible to carry out the work at an elevated temperature.

As soon as the final bending has been accomplished by reswelling between the two mold members 1, 2, the water is discharged from vessel 5; the board including the mold is now located in a suitable drying oven where it is maintained at a temperature of 100-200° C. until the wood is practically dry.

Hereupon the bent board is removed from the bending apparatus by unscrewing the bolts. It now represents the finished article.

Instead of swelling the bent article by imbibition with water solutions may be used imparting to the wood specific desired properties, for instance, strength and hardness.

The bent board may also be impregnated in the manner disclosed in my former application, Ser. No. 527,505, with solutions of thermosetting resins and hardened to transform the soluble resin into its final insoluble state; it may be advantageous to raise the drying temperature in order to accelerate the process; in this way it is possible to produce in one operation hardened bent pieces of balsawood.

The bending operation may be combined in this manner with the introduction of disinfecting, sterilizing, mildew and pest proof substances, coloring agents or products which impart to the wood one or more specific properties.

Any liquid may be used for this purpose provided that it is not repulsed by the wood; it is advisable to use solutions of the impregnating materials in liquids which easily penetrate into the wood. If, for instance, it is intended to impregnate the wood with an oily substance, such as linseed or tung oil, the oils are dissolved in liquids, for instance alcohol, ether or acetone, and incorporated into the compressed wood with or without the addition of hardeners or other substances which are soluble in the solvent. The bending operation is in no way changed or influenced by the impregnation; only the drying may be varied in accordance with the special character of the substances or solutions used.

The invention is described in this specification by way of example only, and it is fully understood that changes and deviations thereof may be made in accordance with individual requirements within the scope of the appended claims.

I claim:

1. Method for the manufacture of a curved workpiece from corkwood comprising compressing a sheet thereof, slowly bending same to curved formation short of its final curved shape, confining said bent sheet between spaced shape-confining faces having the desired curved shape of the finished article and while so confined, imbibing said sheet, reswelling same to occupy the space between said faces, to form a curved workpiece and drying the thus produced curved workpiece while maintaining the same between said space confining faces.

2. Method for the manufacture of a curved workpiece from corkwood comprising compressing a sheet thereof to about one fifth to one tenth of its original thickness, slowly bending same to curved formation short of its final curved shape, confining said bent sheet between spaced shape-confining faces having the desired curved shape of the finished article and while so confined, im-

7  
bibing said sheet, reswelling same to occupy the space between said faces, to form a curved workpiece and drying the thus produced curved workpiece while maintaining the same between said space confining faces.

3. Method for the manufacture of a curved workpiece from corkwood comprising compressing a sheet thereof, slowly bending same to curved formation short of its final curved shape, confining said bent sheet between spaced shape-confining faces having the desired curved shape of the finished article and while so confined imbibing said sheet with an aqueous solution of thermosetting resins, reswelling same to occupy the space between said faces, to form a curved workpiece and drying the thus produced curved workpiece while maintaining the same between said space confining faces.

4. Method for the manufacture of a curved workpiece from corkwood comprising compressing a sheet thereof, slowly bending same to curved formation short of its final curved shape, confining said bent sheet between spaced shape-confining faces having the desired curved shape of the finished article and while so confined imbibing said sheet with an aqueous solution of sterilizing substances, reswelling same to occupy the space between said faces to form a curved

workpiece and drying the thus produced curved workpiece while maintaining the same between said space confining faces.

5. Method for the manufacture of a curved workpiece from corkwood comprising compressing a sheet thereof, slowly bending same to curved formation short of its final curved shape, confining said bent sheet between spaced shape-confining faces having the desired curved shape of the finished article and while so confined, imbibing said sheet with an aqueous solution of thermosetting resins and reswelling same to occupy the space between said faces, to form a curved workpiece and hardening the same at a temperature of between about 100 to 120° C. while maintaining the same between said space confining faces.

FREDERICK F. POLLAK.

#### REFERENCES CITED

20 The following references are of record in the file of this patent:

#### UNITED STATES PATENTS

| 25 Number | Name   | Date          |
|-----------|--------|---------------|
| 2,081,638 | Owens  | May 25, 1937  |
| 2,199,268 | Miller | Apr. 30, 1940 |